

Nov. 5, 1935.

N. F. BEACH ET AL

2,019,648

MOISTUREPROOF CELLULOSE ACETATE SHEETING

Filed July 17, 1931

Fig.1.



Fig.2.



Fig.3.



Inventors

Norman F. Beach & James G. McNally,

By *Newton M. Purvis*  
*Daniel J. Mayne* Attorneys

## UNITED STATES PATENT OFFICE

2,019,648

MOISTUREPROOF CELLULOSE ACETATE  
SHEETINGNorman F. Beach and James G. McNally,  
Rochester, N. Y., assignors to Eastman Kodak  
Company, Rochester, N. Y., a corporation of  
New York

Application July 17, 1931, Serial No. 551,490

13 Claims. (Cl. 91—70)

This invention relates to the manufacture of thin cellulosic acetate sheeting and more particularly to a waterproof and moistureproof sheeting having superimposed thereon separate layers 5 of gum and wax.

It is known to coat paper, cloth, and other forms of cellulosic material with waxes or gums for the purpose of rendering them impenetrable or impermeable to water and other liquids. So far as we are aware, however, there has been no attempt to waterproof or moistureproof cellulose acetate sheeting by the method hereinafter described. The present invention is not concerned broadly with either waterproofing or moistureproofing, but relates to the treatment of a colloidized cellulosic base sheet and involves the use of a type of coating material which, due to its peculiar properties, requires a special technique. The resulting moistureproof coating not only differs from known coatings in the requirements with respect to its mode of application, but also differs in composition in that it contains only two necessary ingredients and does not require the presence of a base material such as cellulose nitrate, cellulose acetate or other cellulose esters or ethers.

Thin cellulose acetate sheeting has found wide use as wrapping or packaging material, due to the fact that it is comparatively tough, flexible, 30 transparent, and impermeable to dust and similar foreign matter. Its principal drawback for this purpose is that, as ordinarily produced, it is not waterproof or moistureproof, and, for this reason cannot be used for wrapping products where substantially complete exclusion of moisture is important. For example, untreated cellulose acetate sheeting of the order of ".001" in thickness will transmit as much as 1.0 to 1.5 milligrams of water vapor per sq. cm. per hour. The 35 improved product which is the subject of the present invention, however, will in some cases transmit as little as .002 milligrams of water under the same conditions, thus showing a marked improvement in water-resistant properties over untreated sheeting.

The principal object of our invention is to produce a highly waterproof and moistureproof form of thin cellulose acetate sheeting. A further object is to provide a wrapping or packaging material which is not only highly water-resistant but is also transparent, flexible, odorless, and non-tacky. Another object is to provide a simple but effective method for moistureproofing thin cellulose acetate sheeting, while at the same time preserving its flexibility, transparency, and

other essential and valuable properties. Other objects will appear hereinafter.

These objects are accomplished by the following invention which in its broadest aspect may be said to comprise applying to a thin base sheet 5 of cellulose acetate a first coating of a gum or resin and then applying a second coating of wax. These materials are preferably applied in the form of solutions in suitable solvents or they may be applied in a molten state, in separate 10 layers, the gum or resin layer in either case being applied first to form a strongly adhering coat followed by the wax coating which, in turn, is strongly held by the gum or resin coat. The sheet may be coated on one or both sides. In 15 case it is to be coated on two sides, this may be accomplished in successive operations, or both sides may be coated simultaneously with a given solution, as will more fully appear in the following description in which reference is made to 20 the drawing forming a part of this application.

In the drawing,

Figure 1 is a diagrammatic representation of one form of apparatus for carrying out the invention, in which the sheet is coated on one side 25 with successive layers of coating material.

Figure 2 is a diagrammatic representation of apparatus similar to, and for use in connection with, that of Figure 1 when it is desired to coat 30 both sides of the sheet.

Figure 3 is also a diagrammatic representation of the equipment for simultaneously coating both sides of the sheet.

We may employ a large variety of gums or resins for forming the gum coating, typical examples of these materials being ester gum, dammar, 35 rosin, and sandarac. Natural or synthetic gums or resins are equally desirable for this purpose. Any of these gums or resins may be used alone or in combination with one another or with many 40 other gums or resins of this general nature which are known to those skilled in the art. The gum must, of course, adhere well to the base sheet and must hold the wax coating without separation.

The wax coating may consist of paraffin, 45 ceresin, beeswax, pimela, lanolin, spermaceti, Montan, bayberry, halowax, japan, candelilla, Chinese wax and other similar waxes, any of which may, as in the case of the gums, be used separately or in combination with one another.

Our invention is distinguished by the application of two or more layers of waterproofing material, the first of which is a gum or resin 50 which adheres closely to the base sheet by virtue 55

of its adhesiveness with respect to cellulose acetate, while the second layer of wax adheres closely to the gum or resin layer due to the mutual adhesion between the gum and wax. The second coating may also consist of a mixture of a gum and wax, the wax preferably predominating. Either or both the gum and wax may for convenience of application be dissolved in a suitable solvent. When coating gums from solution we prefer to use a solvent such as toluene, benzene, xylene, naphtha, gasoline, carbon tetrachloride, ethylene dichloride, and trichlorethylene, or similar solvents, it only being necessary in choosing the solvents to select one which is a good solvent for the gum, but substantially a non-solvent for cellulose acetate. A liquid possessing any appreciable solvent power for cellulose acetate would not be desirable, since it would have a tendency to dissolve and weaken the base sheet during coating and thereby render it unfit for use.

With regard to wax solvents, it may be said that the hydrocarbons such as gasoline, kerosene, petroleum ether, and other compounds of this general nature are preferable. Inasmuch as the wax coating is superimposed on the gum or resin coating, the same care in the selection of the solvent is unnecessary, since the first adhesive coating of gum protects the cellulose acetate sheet to a certain extent from the action of the solvent which may be used in the wax solution. It is necessary, however, to select a solvent which has no pronounced solvent action on the gum, as otherwise the gum coating would be dissolved from the base sheet.

As indicated above, the gum and wax need not necessarily be put into solution, although from the standpoint of convenience in handling they can be more readily and conveniently applied in this way. If desired, each of these materials may be liquefied and applied in a molten condition. In some cases it may be an advantage to carry out the operation in this way, since less complicated drying apparatus is required and the drying time may be somewhat shorter.

The properties of the finished product, such as waterproofness, moistureproofness, flexibility, and transparency, may be controlled within certain limits in accordance with the particular qualities desired, by varying the amounts of gum and wax making up the composite coating. With regard to the waterproofing properties of the coating, it may be stated that, in general, the higher the proportion of wax to gum or resin, the greater will be the water resistant properties, although it is necessary to control the amount of wax in such a way that the transparency of the original acetate sheet is not adversely affected. We have found that if too thick a coating of wax is applied, the material will have a tendency to feel greasy and show finger marks readily. On the other hand, if the proportion of gum is too high, the material will be objectionably tacky. It should be understood, however, that as a general rule the more resinous material present, the better will be the adhesion properties of the composite coating.

In the following examples we have set forth examples of a typical gum, a typical wax solution, and a typical combination gum-wax solution, respectively, but it is to be understood that these formulae are merely illustrative and are not intended as a limitation of our invention, since it will be obvious to those skilled in the art that a larger variety of similar compositions

may be made up in accordance with the present description.

*Example of typical gum-containing solution*

|                                                    | Percent by weight | 5 |
|----------------------------------------------------|-------------------|---|
| Ester gum                                          | 1                 |   |
| Solvent { 80% toluene<br>20% ethylene dichloride } | 99                |   |

*Example of typical wax solution*

|                                                           | Percent | 10 |
|-----------------------------------------------------------|---------|----|
| Paraffin wax                                              | 1       |    |
| Petroleum distillate boiling between 60° C.<br>and 70° C. | 99      |    |

*Example of typical gum wax solution*

|                     | Percent | 15 |
|---------------------|---------|----|
| Paraffin 3½ parts   | 1       |    |
| Ester gum 1 part    |         |    |
| Ethylene dichloride | 15      | 20 |
| Toluene             | 84      |    |

Referring to the drawing in detail, in Figure 1, the numeral 1 designates a thin base sheet of cellulose acetate which is fed from a supply roll 2 between subbing roll 3 and squeeze roll 4. Roll 3 normally dips in a bath of coating fluid 4' contained in vat 5 which may be supplied with a steam jacket or steam coils (not shown) for the purpose of maintaining the coating material in a fluid condition. The numeral 6 designates a drying chamber which is preferably provided with suitable means (also not shown) for maintaining the desired temperature and for removal of solvent vapors. The numeral 7 indicates a second subbing roll having positioned thereover and cooperating therewith squeeze roll 8. Roll 7 is normally partially immersed in a second bath of coating solution 9 contained in vat 10, which, as in the previous case may be provided with known means for maintaining the coating material in a fluid condition. Numeral 11 designates a drying chamber similar to chamber 6. Numeral 12 is a guide roll over which the sheet 1 passes to wind up roll 13.

Figure 2 shows additional apparatus for use in connection with the equipment shown in Figure 1, 14 being a guide roll over which the sheet 1 passes to a subbing roll 15 having positioned thereover and cooperating therewith squeeze roll 16, the function of rolls 15 and 16, as well as 19 and 20, being the same as rolls 3 and 4, and 7 and 8, respectively, of Figure 1. The vats 18 and 22 also serve a purpose similar to that of 5 and 10. In like manner, drying chambers 23 and 24 operate in a manner similar to drying chambers 6 and 11. Numeral 25 designates a guide roll over which the finished sheet passes to windup roll 26.

Figure 3 shows an optional form of equipment for simultaneously coating both sides of a base sheet with a series of waterproofing materials according to the invention. Numeral 27 designates a supply roll from which the base sheet 1 is passed over guide roll 28. Numeral 29 represents an immersion roll normally partially immersed in coating fluid 30 contained in vat 31. Numerals 32 and 33 designate a conventional form of scraping device for removing excess coating fluid from the sheet and insuring uniform application. Numeral 34 is a guide roll over which the sheet 1 passes to drying chamber 35 which is similar in all respects to the drying chambers described in connection with Figures 1 and 2. Numerals 36, 40, and 42 are guide rolls over which the sheet 75

passes in its course to the windup roll 43. Immersion roll 37, vat 38, fluid 39, and drying chamber 41, perform the same functions as the corresponding devices shown in the left-hand portion of Figure 3.

Assuming the operation to be carried out employing the apparatus of Figure 1, the base sheet 1 of untreated cellulose acetate fed from supply roll 2, passes between rolls 3 and 4, roll 3 picking up the gum coating fluid 4\* and carrying it onto the under surface of the base sheet. Roll 4 squeezes off the excess fluid which eventually returns to the bath. The sheet then passes through the drying chamber 6 where the material applied is merely dried at the proper temperature. The second layer of wax is applied from bath 9 in a similar manner by means of rolls 7 and 8, dried in drying chamber 11, passed over guide roll 12, and finally wound up on roll 13. If it is desired to coat both sides of the sheet, instead of being wound up on roll 13, the sheet may be passed around another guide roll 14, thence first through a gum coating operation between rolls 15 and 16, then through a wax coating operation between rolls 19 and 20, and finally wound up upon roll 26, drying of the sheet being accomplished by passage through drying chambers 23 and 24 as in the case of the single coating process of Figure 1.

If it is desired to apply a gum coating to both sides of the sheet simultaneously, the apparatus of Figure 3 may be employed. In this case the sheet 1, fed from supply roll 27, passes over guide roll 28, immersion roll 29, between scrapers 32 and 33, over guide roll 34 and thence to drying chamber 35. During the passage of the sheet over roll 29, the vat 31 is raised to the proper height which places the roll well beneath the surface of the fluid 30 with the result that the coating liquid flows freely into the opening between the down-coming and up-going portions of the sheet, thereby insuring application of the material to both sides thereof at the same time. Excess fluid is removed by scraper bars 32 and 33 which also assist in an even distribution of the material over the surface of the sheet. The single coated sheet is then dried at the proper temperature by passing through drying chamber 35 and is then subjected to a coating of wax by passage through bath 39, roll 37 and drying chamber 41 performing the same functions as previously described, and the finished sheet is finally wound up on roll 43.

It is to be understood that the apparatus herein described is intended to be merely illustrative and that many changes may be made therein without in any way departing from the scope of our invention. It is conceivable that other types of apparatus might be used with equally desirable results in carrying out our process. In fact, the particular apparatus shown and described herein does not of itself form any part of the invention and is intended to be merely conventional.

As illustrating the highly desirable results to be obtained by the use of our process, the following typical examples of coating operations are given below.

#### Example I

A gum solution consisting of  $\frac{1}{4}\%$  ester gum in toluene was applied by immersion to a base sheet of cellulose acetate of about  $.001''$  thickness having an original capacity for transmission of water of 1.0 to 1.5 milligrams per square centimeter per hour. After drying at a temperature of 50-105°

C., a second coating of solution consisting of  $\frac{1}{4}\%$  of a 139° paraffin, dissolved in a commercial hexane having a boiling point of 60 to 70° C. was thereafter applied in the same manner, the sheet being dried at 50 to 105° C. The coated sheet was found to transmit only .005 milligrams per square centimeter per hour. 5

#### Example II

A solution containing 1% ester gum dissolved 10 in toluene was applied by a subbing operation to a cellulose acetate base sheet similar to that used in Example I. After drying at a temperature of 50 to 105° C. a second solution containing 3½% candelilla wax dissolved in gasoline was applied in the same manner as the gum solution and dried at the same temperature as before. The sheet was found to transmit only .026 milligrams of water per square centimeter per hour. 15

#### Example III

A base sheet of cellulose acetate having a thickness of the order of  $.001''$  was coated with a solution consisting of 2% copal dissolved in a solvent consisting of 85% toluene and 15% ethylene 25 chloride. After drying at a temperature of above 50° C., the sheet was coated with a second solution consisting of 5% of a 139° paraffin dissolved in a commercial hexane having a boiling point of 60° to 70° C. After drying, the double coated sheet 30 was found to transmit only .004 milligrams of water per square centimeter per hour.

It is a feature of our invention that the double coating of the sheet as it emerges from the bath of wax solution may, if desired, be subjected to a 35 temperature during the last drying operation sufficient to cause the gum and wax layers to unite or coalesce at their mutual boundary with the result that the coating will range all the way from 100% wax at the outside to 100% gum at the 40 portion in contact with the base sheet.

The double coated product of our invention is readily susceptible to heat or solvent sealing. For example, when two sheets are brought together with their coated surfaces in contact, an effective seal therebetween may be made merely by the application of heat and pressure, the respective moistureproof coatings readily softening and flowing together to form a satisfactory joint at the points of contact. The application of pressure will enhance the coalescing effect produced by the heat and serve to bring the sheets into even closer relation and cause them to adhere strongly to one another. 45

While we prefer to use a base sheet having 55 a thickness of the order of  $.001''$ , it is entirely feasible to moistureproof sheeting of much greater thickness or even of less thickness. Furthermore, the thickness of the respective gum and wax layers may be varied as desired, although 60 we have found it preferable to keep the total thickness of the moistureproofing layer somewhere in the vicinity of  $.00001''$ .

Optional ingredients which may be incorporated into either or both layers making up the water- 65 proof coating, although not in any way essential to the purpose of our invention, are plasticizers such as tricresyl phosphate, triphenyl phosphate, benzyl benzoate, and other plasticizing or softening agents. Furthermore, various spirit- and oil-soluble dyes, aluminum flake, gold leaf, pearl essence, and other coloring materials may be included in the composition, or may be incorporated directly into the original ester dope from which 70 the base sheet is produced. Perfumes or flavoring 75

material may be used, depending upon the use to which the finished product is ultimately to be put. Likewise various ultra-violet filters, such, for example, as those described in the co-pending application of Richardson and Staud, Serial No. 457,508, filed May 29, 1930, may be advantageously used in the manufacture of moistureproof sheeting which is to be used for the wrapping of delicately tinted articles which have been dyed with dyes which are fugitive to ultra-violet light.

It has also been found that the waterproof sheeting of our invention is readily susceptible of being united or joined by applying various solvents to the portions of the material it is desired to unite and bringing them into close contact. As in the case of simple heat sealing, such as described above, heat and pressure are advantageously used to cause those portions of the moistureproof surface which have been softened or partially dissolved by the solvents to coalesce and, upon evaporation of the solvent, to form a strong, uniform, and transparent joint or seal. The heat evaporates off the solvent and leaves only the mingled or coalesced portion of the coatings of the respective sheets adhering and thereby forming a uniform bond between them.

Among the solvents which have been found suitable for the purpose of solvent sealing may be included alcohols of both the aliphatic and aromatic series and containing one or more hydroxyl groups such as methyl, ethyl and normal butyl alcohol, glycerol, benzyl alcohol and cyclohexanol; derivatives of alcohols, such as esters of mono- or polyhydric alcohols, typical examples of which are ethyl acetate, monacetin and diacetin, respectively; keto alcohols, such as diacetone alcohol; aromatic ketones, such as acetophenone, benzophenone, and cyclohexanone; mixed ether-esters of aromatic or aliphatic acids, such as ethoxy ethyl phthalate, mixed ether alcohols, such as the monobutyl ether of ethylene glycol and the monoethyl ether of ethylene glycol; diacyl derivatives of dihydroxy alcohols, such as glycol diacetate; monoacyl derivatives of the monoalkyl ethers of glycol, such as derived from the monoethyl ether of ethylene glycol and others. The discovery that the above mentioned compounds may be used for this purpose is not to be understood as forming part of our invention, since this is the invention of C. J. Staud and William O. Kenyon, as set forth in their Patent No. 1,925,509.

It is to be understood that the terms gum and resin are used herein and in the claims interchangeably and when reference is made to a gum it is to be taken for the purposes of our invention as also including both natural and synthetic materials.

Furthermore, although the specific examples above given are directed to, and the foregoing specification is chiefly concerned with, sheeting composed of cellulose acetate, it is to be understood that we are not to be limited thereby, as our invention is applicable to thin sheeting composed of any cellulosic material to which a gum-wax coating will adhere well, such, for instance, as cellulose acetate propionate, cellulose acetate butyrate, cellulose propionate or butyrate, or that cellulosic material which is commonly known as viscose or regenerated cellulose. The term "cellulosic material" is intended to include all forms of colloidized cellulosic materials ordinarily employed in this art.

Having now particularly described our invention, what we claim as new and desire to secure by Letters Patent of the United States is:

1. The process of moistureproofing thin, flexible, transparent cellulose acetate sheeting adapted for wrapping purposes which comprises first applying thereto an adhesive layer essentially consisting of gum and thereafter superimposing on said gum layer a second layer consisting predominately of wax. 5

2. The process of moistureproofing thin, flexible, transparent cellulose acetate sheeting adapted for wrapping purposes which comprises 10 applying a layer essentially consisting of gum to the sheeting, drying the coating thus formed, thereafter applying a coating consisting predominately of wax, and subjecting the double coating thus formed to a temperature sufficient 15 to cause at least partial coalescing of the gum and wax layers.

3. The process of moistureproofing thin, flexible, transparent cellulose acetate sheeting adapted for wrapping purposes which comprises 20 applying to the sheeting a thin coating essentially consisting of a gum or resin in a molten condition and thereafter superimposing a coating consisting predominately of wax on said first coating. 25

4. The process of moistureproofing thin, flexible, transparent cellulose acetate sheeting adapted for wrapping purposes which comprises applying to the sheeting a thin coating of ester gum in a molten condition, applying sufficient heat to dry the coating thus produced, and applying on the first coating a second coating of molten paraffin. 30

5. The process of manufacturing thin cellulose acetate sheeting of a thickness of the order 35 of .001" which comprises first applying to an untreated cellulose acetate base sheet a solution comprising 1% of ester gum dissolved in a solvent consisting of 80% toluene and 20% ethylene dichloride, subjecting the sheet to a temperature 40 of 50-105° C. for a length of time sufficient to evaporate off the solvents and leave a gum coating closely adhering to said sheet, and thereafter applying to said gum coating a solution comprising 1% paraffin dissolved in a petroleum distillate boiling between 60° and 70° C., and evaporating off the solvent. 45

6. The process of moistureproofing thin, flexible, transparent cellulose acetate sheeting adapted for wrapping purposes which comprises 50 first applying to the surface of the sheeting a thin coating essentially consisting of gum and thereafter superimposing on said gum coating a coating comprising a mixture of a gum and wax. 55

7. The process of moistureproofing thin, flexible, transparent cellulose acetate sheeting adapted for wrapping purposes which comprises first applying to the surface thereof a thin coating essentially consisting of gum and thereafter superimposing on said gum coating a second coating comprising a mixture of a gum and wax in which the wax predominates. 60

8. An article of manufacture comprising a thin, flexible transparent sheet of cellulose acetate adapted for wrapping purposes of a thickness of about .001" having closely adhering to the surface thereof a layer of ester gum, said layer having superimposed thereon and adhering thereto an outer layer consisting predominately of paraffin. 65

9. An article of manufacture comprising a thin, flexible, transparent sheet of cellulose acetate adapted for wrapping purposes having a closely adhering coating essentially consisting 75

of a gum, said gum coating having superimposed thereon and adhering thereto an outer coating consisting predominately of wax.

10. An article of manufacture comprising a thin, flexible, transparent sheet of cellulose acetate adapted for wrapping purposes having a thin, closely adhering coating essentially consisting of gum, said gum coating having superimposed thereon, and adhering thereto, an outer coating comprising a mixture of a gum and a wax.

11. An article of manufacture comprising a thin, flexible, transparent sheet of cellulose acetate adapted for wrapping purposes having a thin, closely adhering coating essentially consisting of gum, said gum coating having superimposed thereon and adhering thereto an outer

coating comprising a mixture of a gum and a wax in which the wax predominates.

12. The process of moistureproofing sheeting composed of thin, flexible, transparent cellulosic sheet material adapted for wrapping purposes which comprises first applying an adhesive layer essentially consisting of gum and thereafter superimposing on said gum layer a second layer consisting predominately of wax.

13. An article of manufacture comprising a thin, flexible, transparent sheet of cellulosic material adapted for wrapping purposes having a closely adhering coating essentially consisting of a gum, said gum coating having superimposed thereon and adhering thereto an outer coating consisting predominately of wax.

NORMAN F. BEACH.

JAMES G. McNALLY